# EUROPEAN PATENT SPECIFICATION

(11) **EP 0 048 083 B1**
(45) Date of publication and mention of the grant of the patent: **05.03.1986**
(21) Application number: 81303264.6
(22) Date of filing: 16.07.1981
(51) Int. Cl.: C23C 4/18, C23C 12/00, C23C 28/00, B05D 1/00, B05D 1/08

(54) **Surface treatment method of heat-resistant alloy**
Verfahren zur Oberflächenbehandlung einer hitzebeständigen Legierung
Procédé pour le traitement de la surface d'un alliage réfractaire

(30) Priority: 17.09.1980 JP 128738/80
(43) Date of publication of application: 24.03.1982
(73) Proprietor: MITSUBISHI JUKOGYO KABUSHIKI KAISHA, Tokyo 100 (JP)
(72) Inventor: Harada, Yoshio Takasago Technical Institute, 2-chome, Arai-cho Takasago-shi Hyogo-ken (JP); Nakamori, Masaharu Takasago Tech. Institute, 2-chome, Arai-cho Takasago-shi Hyogo-ken (JP); Saika, Keigo Takasago Technical Institute, 2-chome, Arai-cho Takasago-shi Hyogo-ken (JP); Fukue, Ichiro Takasago Technical Institute, 2-chome, Arai-cho Takasago-shi Hyogo-ken (JP); Takaoka, Shigefumi Takasago Tech. Institute, 2-chome, Arai-cho Takasago-shi Hyogo-ken (JP); Maekawa, Atsushi Takasago Techn. Institute, 2-chome, Arai-cho Takasago-shi Hyogo-ken (JP)
(74) Representative: Rushton, Ronald

## Description

This invention relates to a method of surface treatment of a member of heat-resistant alloy for use in turbines, blowers, boilers or the like to render it resistant to high temperature oxidation as well as to high temperature corrosion.

In industrial gas turbines using petroleum or natural gas as the fuel, gas temperature at the turbine inlet tends to become higher as the turbine efficiency is improved. On the other hand, as the available fuel supply has changed for the worse in recent years, the fuels used for the turbines have been diversified and the content of corrosive impurities in the fuels such as sulphur (S), sodium (Na), vanadium (V), and so forth has tended to increase. As a result, so-called "hot parts" such as the blades and burners of turbines, that are exposed to these high temperature gases, are subjected to extremely severe high temperature oxidation as well as high temperature corrosion.

These hot parts have conventionally been made primarily of heat-resistant alloys. In particular turbine blades consist of Ni- and Co-based alloys called "super-alloys". However, since high temperature strength is generally a top priority requirement for these super-alloys, they have the drawback that their corrosion resistance and oxidation resistance are not satisfactory. Various attempts have therefore been made to provide these heat-resistant alloys with oxidation resistance and corrosion resistance and various surface treatment methods using for example chemical and physical techniques have been employed. However, none of these methods has been really satisfactory as regards efficiency and cost.

The present invention is directed to-providing a method which overcomes the deficiencies of these previous methods.

In GB-A-2009251 there is disclosed a method of applying a protective coating to a heat resistant alloy part of a kind having at least at its surface an inhomogeneous morphology which involves depositing a first coating of Ni with some Cr (namely 5-15% by weight Cr) for example, it is suggested, by plasma spraying to form a first layer, and then depositing a second coating for example, it is suggested, by slurry aluminising to form a second, aluminised, layer, and thereafter heat treating the part, whereby, it is said, the aluminised layer is caused to diffuse completely through the first layer and into the base material.

In order to provide a member of heat-resistant alloy with high temperature oxidation resistance and high temperature corrosion resistance, the present invention provides a surface treatment method of a heat-resistant alloy comprising the steps of plasma spraying a Ni-Cr alloy on to the surface of a member made of heat-resistant alloy, applying thereon a coating slurry containing aluminium particles and then heat treating the coated member for diffusion penetration which is characterised in that the Ni-Cr alloy comprises 50Ni-50Cr alloy and in that the coating slurry contains additionally Si0₂ particles.

The surface treatment method of the present invention provides the characterizing features as illustrated in Table 1 in comparison with some conventional methods.

The present invention will now be described in more detail by reference to an example in accordance therewith.

A substrate of Udimet 520 (Registered Trade Mark) comprising by weight 19% Cr, 12% Co, 6% Mo, 3% Ti, 2% Al, 1% Fe, Ni-Bal, and widely used as a super-alloy for the hot parts of a gas turbine, was treated in the following sequence: -
(1) After the surface of the substrate had been cleaned with an alkaline emulsion cleaning agent, steam cleaning was carried out using a Fluron type solvent. The surface was further blasted using an Al₂O₃ blast.
2. A Ni-Cr (50/50 by weight) alloy was applied as a coating to form a first layer having a thickness of about 50 pm by plasma spraying.
(3) The surface of the sprayed-on first layer was blasted using Al₂O₃ to remove any oxide film formed on its outermost surface.
(4) The surface of the sprayed-on first layer was coated by spraying on a coating slurry formed by dispersing AI and Si0₂, each having a particle size of about 0.1 to 1 pm, in an organic carrier (alcohol, solvent naphtha, etc.) to form a second layer.
(5) After these treatments, the substrate was placed in an electric furnace and was held at 80°C (±5°C) for 20 minutes to evaporate and remove the liquid. After being further held at 330°C (±5°C) for 15 minutes, the substrate was withdrawn from the furnace.
(6) The substrate was held at 1,080°C for 4 hours inside a hydrogen furnace, was cooled in the furnace and was then withdrawn.

Above mentioned step (4) could be carried out using a mixture of AI with Si0₂ in a mixing ratio by weight of 80/20 or 50/50. Also step (6) could be carried out using a vacuum furnace in place of the hydrogen furnace.

Although in this example Udimet 520 has been treated by the method of the invention by way of example, similar excellent results can also be obtained when treating the surfaces of other substrates such Ni-based alloy, Co-based alloy and stainless steel.

The coated surface of the substrate provided by the above described method had an extremely smooth and flat surface and AI and Si from the second layer sufficiently penetrated by diffusion into the first layer, thereby completely eliminating the fine pores of the first layer. Hence, the composite coating was rendered wholly homogeneous. In other words, since the melting point of AI is 660°C, AI was fused due to the heat-treatment and penetrated into the fine pores, thus presumably rendering the surface smooth and flat. Further, it was confirmed that a part of AI and Si reached and was diffused also into the substrate.

Table 2 illustrates the results of fly-ash errosion resistance test, corrosion resistance test, and practical application test using gas turbine blades, each test being applied to a member treated by a method in accordance with the present invention and a member treated-by a conventional method. The composite coating produced by the method in accordance with the present invention had a better performance in comparison with that produced by the conventional method in the fly-ash errosion resistance test and the corrsion resistance test. In the practical application test using gas turbine blades, too, the coated blade produced using the method of the present invention exhibited the tendency that the deposition amount of the fuel ash become smaller. In a thermal inpact test comprising holding the testpiece at 1,100°C for 15 minutes, then charging it into the water at 20°C and repeating these procedures five times, the composite coating produced by the method of the present invention did not suffer peeling or cracking and had extremely good adhesion.

## Claims

1. A surface treatment method of a heat-resistant alloy comprising the steps of plasma spraying a Ni-Cr alloy on to the surface of a member made of heat resistant alloy, applying thereon a coating slurry containing aluminium particles and then heat treating said coated member for diffusion penetration, characterised in that the Ni-Cr alloy comprises 50Ni-50Cr alloy and in that the coating slurry additionally contains Si0₂ particles.

2. A method according to Claim 1, characterised in that said aluminium and Si0₂ particles have a particle size of about 0.1 µm to 1 pm.

3. A method according to Claim 1 or Claim 2, characterised in that the heat treatment includes the step of holding the coated member at about 1080°C.

4. A method according to Claim 3, wherein said step in the heat treatment is preceded by a heating step to evaporate the liquid in the slurry, followed by a heat treatment at about 330°C.

## Patentansprüche

1. Verfahren zur Oberflächenbehandlung einer hitzebeständigen Legierung, umfassend die Schritte des Aufsprühens von Plasma aus einer Chrom-Nickel-Legierung auf die Fläche eines aus hitzebeständiger Legierung hergestellten Elementes, des Aufbringens einer Streichsuspension, die Aluminiumpartikel enthält sowie der anschließenden Wärmebehandlung des gestrichenen Elementes zwecks Diffusionspenetration, dadurch gekennzeichnet, daß die Chrom-Nickel-Legierung eine. 50%-Chrom-50%-Nickel-Legierung ist, und daß die Streichsuspension zusätzlich Si0₂-Partikel enthält.

2. Verfahren nach Anspruch 1, dadurch gekennzeichnet, daß die genannten Aluminium- und SiO₂-Partikel eine Größe von etwa 0,1 pm bis 1,0 um aufweisen.

3. Verfahren nach Anspruch 1 oder 2, dadurch gekennzeichnet, daß die Wärmebehandlung den Schritt des Haltens des gestrichenen Elementes auf etwa 1080 Grad C umfaßt.

4. Verfahren nach Anspruch 3, dadurch gekennzeichnet, daß dem Verfahrensschritt der Wärmebehandlung der Verfahrensschritt einer Erwärmung vorgeschaltet ist, um die Flüssigkeit aus der Suspension zu verdampfen, gefolgt von einer Wärmebehandlung bei etwa 330 Grad C.

## Revendications

1. Procédé pour le traitement de surface d'un alliage réfractaire, au cours duquel on applique par projection au plasma un alliage Ni-Cr sur la surface d'un élément fait de l'alliage réfractaire, on l'enduit d'un coulis de revêtement renfermant des particules d'aluminium, puis on traite thermiquement l'élément ainsi revêtu de manière à produire une pénétration par diffusion, caractérisé en ce que l'alliage Ni-Cr est un alliage 50 Ni-50 Cr, et en ce que ledit coulis de revêtement renferme en outre des particules de Si0₂.

2. Procédé selon la revendication 1, caractérisé en ce que lesdites particules d'aluminium et de Si0₂ ont une taille comprise approximativement entre 0,1 pm et 1 pm.

3. Procédé selon la revendication 1, caractérisé en ce que le traitement thermique comporte une étape de maintien de l'élément revêtu à environ 1080°C.

4. Procédé selon la revendication 3, dans lequel ladite étape du traitement thermique est précédée d'une étape de chauffage pour faire évacuer le liquide du coulis, suivie d'un traitement thermique à environ 330°C.
